

W. D. COOLIDGE.  
COMPOSITE METAL BODY.  
APPLICATION FILED MAR. 19, 1915.

1,162,342.

Patented Nov. 30, 1915.



Inventor:  
William D. Coolidge  
by *Alma A. Davis*  
His Attorney.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## COMPOSITE METAL BODY.

1,162,342.

Specification of Letters Patent. Patented Nov. 30, 1915.

Application filed March 19, 1915. Serial No. 15,464.

*To all whom it may concern:*

Be it known that I, WILLIAM D. COOLIDGE, a citizen of the United States, residing at Schenectady, in the county of Schenectady, 5 State of New York, have invented certain new and useful Improvements in Composite Metal Bodies, of which the following is a specification.

The present invention comprises a metal body consisting of tungsten or molybdenum and a layer of precious metal intimately united therewith which is useful for various purposes in the arts, as, for example, in dentistry, as dental pins or the like. 10 Tungsten and molybdenum although substantially incorrodible are not wet by gold even when care is exercised to prevent oxidation.

I have discovered that when a small amount of platinum is alloyed with the gold, the tungsten or molybdenum is wet by the molten alloy in an atmosphere of hydrogen and a firm union is produced.

My invention comprises a composite body 25 of tungsten or molybdenum joined to a layer of a gold-platinum alloy, as, for example, a rod or wire coated with gold-platinum alloy.

The accompanying drawing shows partly 30 in section a metal article made in accordance with my invention.

This new article of metal may be produced by melting gold containing about 1.5% of platinum in an alumina crucible in a hydrogen atmosphere and dipping the tungsten or molybdenum, for example, as a rod or wire 1 of ductile metal, into the molten alloy. A thin layer 2 of the gold-platinum alloy will unite firmly with the tungsten or 35 molybdenum. The hydrogen not only prevents surface oxidation of the tungsten or molybdenum but also enables the gold alloy to wet or adhere to the surface of the refractory metal. Other alloying metals, such,

for example, as palladium may also be added 45 to the gold alloy to modify its melting point or its hardness.

The gold coated metal article has the mechanical strength of tungsten or molybdenum, and the gold-coated surface is not only 50 incorrodible but may readily be soldered or otherwise joined to other metals. The good mechanical properties of tungsten or molybdenum, particularly toughness and springiness are not lost at the high temperatures 55 necessary for casting or soldering operations, say about 1000 to 1100° C.

While especially useful in dentistry this new metal article is not limited to this particular field. It may be used in the 60 chemical industry or wherever a substantially incorrodible, strong, resilient metal article is desired.

As above indicated, molybdenum is to be considered the equivalent of tungsten for the 65 purposes of the present invention.

What I claim as new and desire to secure by Letters Patent of the United States, is:—

1. A composite metal article comprising tungsten and a coating comprising an alloy 70 of gold and platinum metallically united to or wetting said tungsten.

2. A metal article consisting of ductile tungsten and an adherent layer of an incorrodible alloy consisting largely of gold. 75

3. A composite metal article consisting of a ductile, mechanically strong and resilient metal retaining said properties at a temperature of at least about 1000° C. and a coating 80 of incorrodible alloy comprising gold and platinum adhering to the surface of said metal.

In witness whereof, I have hereunto set my hand this 18th day of March 1915.

WILLIAM D. COOLIDGE.

Witnesses:

BENJAMIN B. HULL,  
HELEN ORFORD.

Correction in Letters Patent No. 1,162,342.

It is hereby certified that in Letters Patent No. 1,162,342, granted November 30, 1915, upon the application of William D. Coolidge, of Schenectady, New York, for an improvement in "Composite Metal Bodies," an error appears in the printed specification requiring correction as follows: Page 1, line 25, for the word "laver" read *layer*; and that the said Letters Patent should be read with this correction therein that the same may conform to the record of the case in the Patent Office.

Signed and sealed this 11th day of January, A. D., 1916.

[SEAL.]

J. T. NEWTON,

*Acting Commissioner of Patents.*

Cl. 29—182.